

Feb. 15, 1938.

W. C. NASH

2,108,231

## METHOD OF MAKING PAPER

Filed March 14, 1935



Inventor.  
William C. Nash  
By: Spec J. Day  
Attorney.

## UNITED STATES PATENT OFFICE

2,108,231

## METHOD OF MAKING PAPER

William C. Nash, Neenah, Wis.

Application March 14, 1935, Serial No. 10,990

2 Claims. (Cl. 92—39)

This invention relates to improvements in a method and means for making paper or board, and refers specifically to a method of applying, during a continuous paper making operation, a liner of fibrous material having predetermined characteristics to a web of fibrous material having different predetermined characteristics.

As described in my United States Letters Patent No. 1,973,722, board or paper having characteristics of heat and sound insulation may be made from kapok fibres. However, as pointed out in said patent, the kapok fibre is very difficult to beat and felt into paper, the resulting paper being very weak and having little or no tensile or impact strength. By the use of the invention described in said patent, the beating and felting problem is solved and the strength of the resulting paper or board is materially increased by the presence of a relatively thin layer of rag or other reinforcing fibre on one face of the paper or board.

As one feature of my present invention, a reinforcing layer or liner of rag or other like fibres may be applied to the product described in my above mentioned patent, that is, to the opposite face of the web of paper or board whereby the strength of the resulting product is materially increased.

The apparatus of my present invention, although ideally adapted for the application of a fibrous layer or liner to a preformed web of paper, may be used with equal facility to apply a coating material or surface layer of other material to a passing web of paper or board.

Other objects and advantages of my invention will be apparent from the accompanying drawing and following detailed description.

In the drawing, Fig. 1 is a fragmentary diagrammatic view of a portion of a paper making machine equipped with suitable mechanism for carrying out my invention.

Fig. 2 is a detailed sectional view of the product of my invention.

Referring in detail to the drawing, 1 indicates a fragmentary portion of a paper making machine such as a Fourdrinier machine altered in accordance with the disclosure in my United States Letters Patent No. 1,973,722. A portion of the machine illustrated in Fig. 1 hereof comprises an intermediate part of the paper making machine. The table portion 2 of said machine may be supported by suitable legs or standards 3 and may carry a series of table rolls 4 over which the Fourdrinier screen or wire 5 passes. As described in my hereinbefore mentioned United

States Letters Patent, a web is formed upon the screen 5 comprising kapok or like fibres and rag or similar reinforcing fibres, the kapok fibres comprising substantially the entire thickness of the resulting web and the rag fibres being present in the form of a relatively thin layer at the lower face of the web. As described in said patent, the layer of rag fibres is utilized as a reinforcing medium for the kapok web inasmuch as pure kapok in felted form has relatively no tensile or impact strength. Hence, the screen 5 is illustrated in Fig. 1 as carrying a web 6 having characteristics similar to the product of the invention comprising the subject matter of my issued patent.

A frame 7 may be mounted above the path of screen 5 and web 6 as the same passes over the table rolls 4, said frame being secured to the table 2 by means of bolts 8 or the like. It is to be understood, of course, that two such frames are provided, one on each side of the paper making machine and as will be hereinafter more fully described, said frames are adapted to support a screen roll 9 which may comprise a cylindrical screen supported upon suitable circular frame members. The roll 9 extends transversely across the paper making machine and is of a length substantially equal to the width of screen 5 and web 6. The lower surface of the roll 9 may be positioned adjacent screen 5, the proximity of said roll with the screen being adjustable.

A rod 10 may be slidably positioned in each of the frames 7, said rods being provided with keys 11 which cooperate with keyways (not shown) provided in collars 12 positioned upon and secured to each of the frames 7. The arrangement is such that rods 10 may be movable upwardly and downwardly but are prevented from rotating. The upper ends of each of said rods 10 are provided with threads 13 and a hub 14 of a hand wheel 15 may engage the threads of each of said rods. A coil spring 16 may encircle an intermediate portion of rod 10 and may be confined between the lower surface of hub 14 and the upper surface of collar 12. The lower end of each of the rods 10 may be threadedly engaged with a nut 17. A cross arm 18 may be rigidly secured at the end of each of the rods 10, and grooved wheels 19 may be journaled as at 20 in each end of each of the cross arms 18. The grooved wheels 19 are similar in structural features to the usual sheave wheel. A pair of rings 21 may be secured to the inner portion of the roll 9 and may be adapted to register with the grooves in wheels 19, the arrangement

being such that roll 9 is suspended upon said wheels.

As can readily be seen the position of roll 9 with respect to screen 5 may be changed by manipulating the opposite hand wheels 15 upon rods 10. By so manipulating said wheels, the compression of springs 16 may be changed to raise or lower roll 9. However, by the provision of springs 16, roll 9 is not positively maintained in its adjusted position since the same is free to move upwardly against the impulse of said springs in the event that incompressible material inadvertently passes between the surface of the roll and the screen. In other words, roll 9 may be positioned upon what is hereinafter termed as a floating support.

A supporting member 18' may be mounted upon each side of the machine frame, said member being provided with arms 19' and 20'. A bolt 21' may be carried by each arm 19' and 20' at the upper ends of which guide rolls or sheaves 22' may be rotatably positioned. A rim 23' may be carried at the extreme ends of the roll 9, said rim being adapted to ride in the grooves of the guide or sheave wheels 22'. Wheels 22', of course, can be adjusted upwardly or downwardly by means of nuts 24'.

A head box 22 may be positioned above table 2 and may transversely span the paper making machine. The box 22 may be provided with compartments 23, 24 and 25, which are adapted to contain a quantity of rag pulp or the pulp of any type of reinforcing fibres. If desired, the box 22 may contain a coating material or other substance which is to be applied to the roll 9 as will be hereinafter described.

Box 22 may be connected to header 26 which is adapted to serve as the supply medium for the roll 9, header 26 being connected at its opposite end to a suitable source of supply of such material. The material passed through header 26 may be initially discharged into compartment 23 and when the level of said material in said compartment raises to the height of partition 27, the material flows over said partition into compartment 24. Both compartments 23 and 24 may be provided with pipes 28 and 29 respectively which are adapted to conduct water or other fluid into the compartments for the purpose of dilution and agitation of the materials in said compartments. When the material within compartment 24 rises above the level of partition 30, said material flows over said partition into compartment 25 which may be of triangular cross section and may be provided with pipe 31. Pipe 31 functions in the same manner as pipes 28 and 29 and is adapted to carry liquid under pressure similar to pipes 28 and 29.

One wall 32 of compartment 25 is hinged or swingably mounted, as at 33, whereby the angular relationship of said side may be changed. An extension 34 may be secured to the outer edge of wall 32 and may extend downwardly toward roll 9. Walls 35 may be carried by the extension 34, the arrangement being such that the material in compartment 25 overflows the end of wall 32 and passes downwardly over extension 34 between walls 35. A rubber apron 36 may be secured to the lower edge of extension 34 and is adapted to ride over the periphery of roll 9 when the same rotates. It can readily be seen that by the provision of the pivotal mounting of wall 32, extension 36 may be changed in position with respect to compartment 25 when roll 9 is moved upwardly or downwardly.

75 In carrying out my invention, an aqueous pulp

of rag or similar fibre may be introduced into box 22 through pipe 26. Said pulp may be passed through compartments 23, 24 and 25, being diluted and agitated by the showers 28, 29 and 31. Eventually the pulp passes over the end of wall 32 and is deposited upon the screen surface of roll 9. The aqueous carrier of the pulp may pass through the screen and may be caught by vat or savall 37 from whence it may be either removed from the system or returned to the weir 10 as make up water, or it can be discharged into the return water on the paper making machine. A web 38 of intermatted fibres may thus be formed upon the surface of the screen and the same may be joined under the pressure of roll 9 to web 6 15 carried upon screen 5. The two webs thus brought into contact adhere to each other and web 38 being materially thinner than web 6 is stripped from the screen surface of roll 9.

Both webs 6 and 38 comprising composite web 20 39 at this period possess a relatively high aqueous content and consequently the fibres of both are in somewhat of a distended condition. Hence, upon further removal of the aqueous carrier from both webs by suction and pressing, the webs are combined or amalgamated as a unitary or integral structure.

The resulting composite web 39, originally comprising a relatively thin liner 40 of rag or other reinforcing fibre and a relatively great thickness 30 41, is now augmented by a second relatively thin liner 42 whereby a paper or board is provided which partakes principally of the characteristics of the kapok 41 supplemented by the strength-giving properties of the liners 40 and 42. 35

It is to be understood, of course, that the concept of my invention is broadly directed to the application of a layer of substantially any type of material to the surface of a continuously passing wet web. For instance, the material passed 40 to box 22 may comprise a coating material comprising the usual mineral coating substances in an aqueous carrier. This material may be carried to the surface of roll 9 and may be carried in a more or less thin film to the surface of the 45 web carried upon wire 5 which in this instance may comprise any type of fibres. In this manner the coating substance may be uniformly applied to the surface of the web. When utilizing a coating material, the mesh of the screen on 50 roll 9 is sufficiently fine, 40 to 60 mesh, taken in conjunction with the viscosity of the coating substance that no material quantities thereof will pass therethrough.

I claim as my invention:

1. In a process wherein a pulp comprising, kapok fibers and fibers having the characteristics of felting into a relatively strong structure is deposited upon a continuously moving foraminated surface to form a composite mat having a 60 lower relatively thick layer of kapok fibers and an upper relatively thin layer of said other fibers, the improvement which comprises, depositing a fibrous pulp comprising fibers having characteristics of felting into a relatively strong structure upon a rotating foraminated surface to form a mat upon said surface, and bonding said mat upon the upper surface of said first mentioned kapok fiber mat under substantially constant pressure, said pressure being self-variable in 70 direct relation to the variations in the aggregate thickness of said composite mat.

2. A process of forming a composite mat having a central relatively thick layer of kapok fibres and an upper and lower relatively thin layer of

fibres having the characteristics of felting into a relatively strong structure which comprises, passing a web including a lower layer of said last mentioned fibres and an upper layer of kapok fibres forwardly on a continuously moving foraminated surface, depositing a fibrous pulp comprising fibres having characteristics of felting into a relatively strong structure upon a rotat-

ing foraminated surface to form a mat upon said surface, and bonding said mat upon the upper surface of the forwardly passing web under substantially constant pressure, said pressure being self-variable in direct relation to the variations in the thickness of the forwardly passing web. 5

WILLIAM C. NASH.